

Oct. 21, 1941.

E. R. DARBY, ET AL

2,260,247

METHOD OF MAKING BEARINGS

Filed Dec. 29, 1939



Fig. 1



Fig. 2



Fig. 3



Fig. 4



Fig. 5



Fig. 6



Fig. 7



Fig. 8

INVENTORS.  
Ernest R. Darby.  
Carlos M. Heath.

BY  
*Cobitt, Milby & Miller*  
ATTORNEYS.

## UNITED STATES PATENT OFFICE

2,260,247

## METHOD OF MAKING BEARINGS

Ernest R. Darby and Carlos M. Heath, Detroit,  
Mich., assignors to Federal-Mogul Corporation,  
Detroit, Mich., a corporation of Michigan

Application December 29, 1939, Serial No. 311,525

4 Claims. (Cl. 29—149.5)

This invention relates to a method of making bearings. More specifically, it deals with bearings having steel backs and copper base alloy linings. It refers in particular to such bearings where the lining is applied in the form of metal powder.

The use of a bronze liner in a steel back as a bearing is not new. The lining bronze has been made of various alloys. One such alloy or class of alloys is copper and lead with the lead content ranging from 20% to 45%. Another alloy is composed of copper and lead with a small percentage of tin. Another alloy is one of copper and lead with a small amount of nickel. Small amounts of silver have been used along with copper and lead.

Bearings with liners of these alloys, as well as others having a copper base, have been made by different methods. One method comprises the pouring of the melted copper base alloy into a heated steel shell in a suitable mold followed by rapid chilling, whereby the alloy is bonded or fused to the steel. Another method comprises the spinning of the melted bearing alloy in the heated shell followed by rapid cooling. Still another method has been used where the bronze or copper-lead bearing metal is melted in a closed tube or shell in a reducing atmosphere and the whole rotated to spin the bearing alloy into position.

Metal powder has been used in the application of the bearing liner to the steel supporting back of the bearing. One method makes use of a powder composed of particles of lead enveloped in a shell of copper. This copper coated lead powder is compressed upon a steel bearing back which has been electroplated or otherwise coated with a thin layer of copper. The powder layer is sintered into position under pressure at relatively high temperature, thereby bonding the particles of powder together and the layer as a whole to the copper plated steel back. Another method employs a mechanical mixture of copper and lead powder or of copper, lead and tin powders. The powder mixture is compressed upon a steel backing which has been coated with a thin lead-tin layer. A very high pressure is used whereby the compressed powder layer imbeds in the lead-tin layer sufficiently to be held in place during handling and sintering. Sintering under pressure at a temperature around 1500° F. affects bonding of the bearing layer to the steel and a union of the metal particles in the bearing layer. Other methods similar in nature have been used and powders of various compositions have been

employed. One composition contains graphite particles along with the copper, tin and lead, and a chemical is frequently added for the purpose of producing porosity which later is supposed to absorb lubricating oil.

All of the bronze or copper-lead lined bearings as herebefore described have characteristics which are more or less undesirable either from a manufacturing standpoint or in actual bearing service. It has been found by experimental tests that the iron which is dissolved into the bronze or the copper-lead when the melted alloy is poured into a steel bearing shell, lowers the bearing properties of the finished bearing. Other impurities dissolve in the bearing alloy during the melting process, and with some melting units and processes it is necessary to add metallic or non-metallic elements or substances known as fluxes to remove gas or oxide and in other manners improve the castability of the melted metal. These fluxes, if allowed to remain in the alloy, are in some instances harmful to bearing performance. The high temperature employed when the melted bearing alloy is cast or spun into position on the steel backing material, necessitates operations which are expensive and, in addition, considerable excess alloy must be removed by subsequent machining operation.

When the bearing metal layer is applied to the steel backing in powder form by pressing the powder upon the steel bearing member followed by sintering under pressure, several serious manufacturing difficulties are encountered. If the powder used be copper coated lead powder and the sintering temperature employed be low enough to prevent lead sweating under pressure, the time necessary to properly bond the particles of powder together and the whole bearing layer to the steel backing is very long and the operation becomes expensive. This is also true when the powder used is a mechanical mixture of copper and lead or of copper, lead and tin, and in this case it is impossible with very high lead mixtures to sinter under pressure without sweating a large amount of lead. If sintering is attempted without pressure being applied at the same time, blistering will occur resulting in excessive porosity and very poor bond or union between the bearing metal layers and the steel back.

We have found that a satisfactory and superior bearing can be made with the use of metal powder whereby the difficulties encountered in other methods are eliminated. In our process we may employ either copper coated lead powder or a mechanical mixture of copper and lead powders

or copper, tin and lead powders. In addition, we may use a mixture of copper coated lead powder and copper or lead powder added for the purpose of controlling the chemical composition. We have also found that small amounts of tin may be added which, under certain conditions, is advantageous to our process.

The accompanying drawing illustrates diagrammatically the steps in the preferred form of our method. In this drawing:

Figure 1 is a section through a portion of an unplated metal backing for the bearing produced by our method.

Figure 2 shows the backing plated with a coating of bonding material.

Figure 3 shows the powdered bearing material applied to the plated bearing backing.

Figure 4 illustrates the first sintering operation.

Figure 5 illustrates a rolling operation which may be performed after the first sintering operation.

Figure 6 is a view similar to Figure 4 illustrating the second sintering operation.

Figure 7 illustrates another rolling operation which may be used.

Figure 8 illustrates the bearing back with the bearing metal applied thereto formed into the desired shape.

By our process, the steel backing member 1 (Figure 1) is electroplated or coated by any convenient method with a coating 2 (Figure 2) of copper, tin or other suitable bonding metal. It is even practical and advisable at times to make use of several of these coatings through electro-deposition. A layer 3 (Figure 3) of the metal powder is then placed on the backing and the bearing blank is sintered in a suitable atmosphere to prevent oxidation, at a temperature of about 1100° F., as indicated in Figure 4. The time of sintering will vary with the thickness of the layer of powder and the thickness of the steel backing member. However, under average conditions, this time should not exceed thirty minutes. After the bearing blank has been sintered, it is cooled to room temperature while still maintaining a reducing atmosphere, and removed from the furnace. It is then put in a suitable die and pressed or rolled between suitable rollers, as indicated in Figure 5, under a pressure between 2500 and 20,000 lbs. per sq. in. depending upon the nature of the powder and the thickness of the layer. This pressing operation serves to compact the metal powder layer without danger of causing blistering or sweating in the sintering operation which is to follow. The bearing blank is then again sintered, as shown in Figure 6, for a period of 10 to 30 minutes in a reducing atmosphere in a furnace held at a temperature not exceeding 1700° F. Cooling is effected as before in the reducing atmosphere.

By the above operation we have provided a bearing blank upon which the copper-lead or bronze layer is securely bonded without danger of lead sweating or blistering during any of the operations. In addition, such a bearing blank is remarkably free from porosity and will require but a slight amount of rolling or pressing before the finishing or machining operations necessary to complete the bearing.

A modification of this method may be employed with a certain type bearing whereby the properly plated steel bearing member is placed in a die and the metal powder as above is compressed upon all surfaces under a light pressure not ex-

ceeding 7500 lbs. per sq. in.; the desired pressure depending upon the density and other characteristics of the powder. This pressing operation serves to densify the metal powder layer to an extent whereby the bearing blank with the powder layer upon it may be handled in subsequent operations. After this pressing operation, the blank is sintered in a reducing atmosphere at a temperature of about 1100° F. and cooled as before mentioned. It is then again compressed in a suitable die under a pressure of from 2500 lbs. per sq. in. to 20,000 lbs. per sq. in. depending upon the thickness of the steel backing and the metal powder layer. Final sintering then follows in a reducing atmosphere at a temperature of about 1700° F., whereby the metal powder layer is bonded to the plated steel backing and the particles of powder are thoroughly united. Cooling is then effected as before in a reducing atmosphere.

Another modification has been found practical with certain types of bearing blanks, wherein the metal powder layer is spread loosely upon the plated steel back and then sintered at a temperature not exceeding 1700° F. The blank is then cooled in a reducing atmosphere as before.

After the bearing blanks have been prepared as above, a pressing operation may or may not be necessary depending upon the density desired in the finished bearing. In the case of the average bearing, such as used in internal combustion engines, a pressing operation is desirable and it has been found that a pressure of as high as 40 T. per sq. in. can be safely applied to the sintered metal surface for the purpose of densification and for the purpose of sizing the blank to the desired thickness. This operation may be a rolling operation, as shown in Figure 7. We have found that by our process this final pressing operation produces a surface which may be used in many applications without any machining. It of course is understood that where the bearing blank has been made in strip or other flat form, a forming operation is required to produce the desired shape, for example, that of Figure 8.

One of the advantages of our method is that the metal powder may be applied as a loose layer on the steel back, and sintered without lateral or longitudinal shrinkage and without the formation of shrinkage cracks in the sintered surface. During our first or low temperature sintering, the particles of powder are slightly knit together and slightly bonded to the plated steel back, but not enough diffusion has taken place to cause appreciable shrinkage of the layer. The pressing operation then so compacts the layer that it can not shrink or crack in final sintering. In fact, a slight expansion is noticeable in the final sintering operation.

The advantages of this process are particularly evident when thick bearing layers are desired and when sintering under pressure causes blistering and lead sweating.

Although we have described our process as using a plated steel backing member, we do not wish to confine ourselves to that alone. It is within the spirit of our invention to use any strong rigid material plated as described or any copper base alloy such as argentiferous copper, bronze, brass or leaded bronze as a backing member.

Having thus described our invention, what we claim is:

1. The method of producing a bearing member which consists essentially in placing a layer of

the bearing-forming metallic material on the back in non-compacted powdered form and then sintering in a non-oxidizing atmosphere at a temperature of from about 1100° to 1700° F. in order to partially bond the particles of non-compacted powder together and the layer as a whole to the back, then pressing or rolling the blank thus formed to compact the sintered layer to eliminate substantially all voids therefrom, again sintering said bearing blank in a non-oxidizing atmosphere at a temperature of from about 1100° to 1700° F. in order to complete bonding of the particles together and the layer as a whole to the back, and cooling in a non-oxidizing atmosphere.

2. The method of producing a bearing member which consists essentially in placing a layer of the bearing-forming metallic material in non-compacted powdered form on the back and then sintering in a non-oxidizing atmosphere at a temperature of from about 1100° to 1700° F. in order to partially bond the particles of non-compacted powder together and the layer as a whole to the back, cooling the blank thus formed in a non-oxidizing atmosphere, then pressing or rolling said blank to compact the sintered layer to eliminate substantially all voids therefrom, again sintering said bearing blank in a non-oxidizing atmosphere at a temperature of about 1700° F. in order to complete bonding of the particles 30

together and the layer as a whole to the back, and cooling in a non-oxidizing atmosphere.

3. The method of producing a bearing member which consists essentially in applying a coating of bonding metallic material to a bearing blank, placing a layer of the bearing-forming metallic material in non-compacted powdered form on the back and then sintering in a non-oxidizing atmosphere at a temperature of about 1100° F. in order to partially bond the particles of non-compacted powder together and the layer as a whole to the back, cooling the blank thus formed in a non-oxidizing atmosphere, then pressing or rolling said blank under a pressure between 2500 and 20,000 pounds per square inch to compact the sintered layer to eliminate substantially all voids therefrom, again sintering said bearing blank in a non-oxidizing atmosphere at a temperature of about 1700° F. and cooling in a non-oxidizing atmosphere.

4. A method according to claim 3 wherein the said bearing blank is subjected to an additional pressing or rolling operation after the second sintering operation under a pressure not exceeding 40 tons per square inch to densify the bearing metal layer and size the blank to the desired thickness.

ERNEST R. DARBY.  
CARLOS M. HEATH.